

## 1

2,938,774

## CHEMICAL MILLING PROCESS

Lowell W. Bahe, Milwaukee, Wis., assignor to Allis-Chalmers Manufacturing Company, Milwaukee, Wis.

No Drawing. Filed Apr. 16, 1958, Ser. No. 728,782

8 Claims. (Cl. 41—42)

This invention relates generally to the controlled erosion of metals and more particularly to a process of chemical milling whereby a finish and depth of cut are readily controlled.

In the arts of fabrication, mechanical milling operations have become very complex when the piece to be milled has an unusual shape, when it is thin and therefore structurally weak, when the area to be milled is located in an almost inaccessible place, when the piece is very hard or soft (tough), and when the piece is very small. In many if not all of these cases, mechanical methods of milling are not completely satisfactory and new methods are needed.

The aircraft industry at the present time has devised a partial solution to the problem with the chemical milling process described in U.S. 2,739,047 for milling aluminum parts having unusual shapes, e.g., air foils and the like, and where excessive weight must be reduced to a minimum. However, that process is not totally suited for the easily oxidized metals, e.g., iron and the like.

At present, no chemical milling process, that is, the dissolution of metal from selected areas (excluding, of course, electropolishing), is known which has been commercially successful in the chemical milling of iron, steel, bronze and brass, the more common of the useful metals. Etching processes are used to engrave metal surfaces, or to reveal microstructures, and pickling is widely practiced, but none of these should be included in the term "milling" when referring to the controlled removal of a specific amount of metal.

In an attempt to find a satisfactory method for effecting the desired chemical action, the prior art has proposed several methods. One such method utilized the common mineral acids which attack iron. However, this method was not a commercial success because the acid attack is not uniform and leaves a pitted and etched surface rather than a smooth shiny surface.

Another prior art proposal for chemically milling iron, steel and the like utilized a solvent consisting of an aqueous system, e.g., sodium hydroxide ( $\text{Na}^+\text{OH}^-$ ). This was also disadvantageous because the aqueous phase provided an electrically conducting path for an anodic-cathodic attack (which is a mechanism of ordinary corrosion) and prevented proper controls from being effected for the process.

Since iron and steel are the most widely used structural materials, a need exists for a process with which these materials may be effectively milled utilizing chemical means. The present invention satisfies this need.

Because of the importance of the irons and steels, the present invention will be described relative to these materials, although it is understood that many of the same considerations will apply equally to other structural materials such as the iron alloys, brass, bronze, copper, zinc, titanium, and even tungsten and molybdenum.

The present invention is predicated upon the discovery of an excellent chemical milling process utilizing a bubbling oxidant, to effect the controlled erosion of metal

## 2

values from iron, steel and like structural materials, and a nonaqueous solvent consisting essentially of phosphorus oxychloride for dissolving the metal values removed from the materials and maintaining the values and the oxidant in a state of solution.

Accordingly, one of the prime objects of the present invention is to provide a chemical milling process which obviates the inherent disadvantages of the prior art systems including the noncontrollable ancillary corrosion attendant to the aqueous mediums with which these prior art systems operated.

Another object of the present invention is to provide a method of chemical milling in which the coaction between a controlled flow of an oxidizing fluid through a nonaqueous solution consisting essentially of phosphorus oxychloride is utilized to control milling depth and to provide an even uniform surface to the metal being processed.

Another object of the present invention is to provide a method for the controlled erosion of metal values from metal stock utilizing a nonaqueous heated solvent consisting essentially of phosphorus oxychloride.

Another object of the present invention is to provide a method for the controlled erosion of metal values from metal stock utilizing a nonaqueous liquid solvent through which is bubbled a controllable stream of a fluid oxidant selected from the group consisting of chlorine, bromine and iodine, whereupon the exposed metal values are removed from metal stock at a rate which is functionally related to the concentration of the oxidant in solution as determined by the controllable rate of flow of the fluid oxidant.

These and still further objects as will appear are fulfilled by the present invention in a manner which is readily discerned from the following detailed description of this invention.

Broadly speaking, the present invention is based upon my discovery that exceptionally fine results are obtained from a chemical milling system having a solvent of phosphorus oxychloride. My process embraces the immersion of cast iron, steel and like materials into the solvent and then bubbling a stream of a fluid oxidizing agent through the solvent to mill the surface of the metal at a controlled rate.

A further aspect of my invention is that it can also be adapted for selective milling or embossing by merely applying a protective coating to those portions of the metal article where milling is not desired. In my quest for a coating which would protect the metal by effectively resisting the action of my milling system, I found that sodium silicate quite unexpectedly provides a coating having all of the aforescribed properties and an excellent mask in the practice of this aspect of my invention. Thus when I selectively paint or coat portions of the metal articles with sodium silicate, the sodium silicate effectively inhibits the milling reaction from affecting the metal over which the sodium silicate is painted.

In one practice of the present invention, a piece of Armco iron is immersed into a heated (90 to 100° C.) phosphorus oxychloride solution. Through this solution I then bubbled a continuous stream of chlorine gas. I permit the action to continue for approximately one hour. During the course of the process, the piece of iron lost 15% of its weight and its thickness decreased about .006 inch. The removal of the iron was quite uniform and the surface appeared very shiny and smooth. The corrosion products dissolved in the hot phosphorus oxychloride but as the phosphorus oxychloride was cooled to about 60° C., the corrosion products precipitated out and were removed from the solution by filtration. The system was then ready for another run.

In another practice of the present invention a piece

of 18-8 stainless steel is immersed into a bath consisting essentially of phosphorus oxychloride which has been heated to slightly over 95° C. A stream of bromine is then directed into the solution with slight agitation or stirring. The rate of corrosion product removal is again approximately .005 inch per hour.

In another practice of the present invention, a piece of 12% chromium steel is immersed into a bath of phosphorus oxychloride which has been heated to at least 90° C. A stream of chlorine was bubbled through the heated bath for about one hour. After an hour, the piece of steel was withdrawn from the system. The product again was found to have very uniform removal and an extremely shiny even surface.

An additional practice of the present invention comprises the immersion of ordinary cast iron into a heated (90-100° C.) bath of phosphorus oxychloride and bubbling a stream of iodine therethrough. Although the bubbling oxidant itself creates sufficient turbulence to provide excellent results and a reasonable rate, it was found that by imparting slight mechanical agitation to the bath while the oxidant is bubbling therethrough, gives equally satisfactory results at a more rapid rate. As in the earlier practice, the cast iron surface was milled at a rate of approximately .005 inch per hour which was maintained fairly uniform over a period of two hours.

The uniformity of depth and finish provided upon the piece was substantially comparable with the other pieces which were milled in accordance with my invention.

A further examination of all the samples prepared in accordance with this invention indicated an average surface roughness of  $5 \times 10^{-6}$  inches (R.M.S.) which in the trade is considered to be an excellent surface finish.

In another practice of the present invention, a design is painted on a piece of Armco steel with a sodium silicate solution. The coated piece is then dried at approximately 110°. When the "painted" piece is dry, it is immersed into a solution of phosphorus oxychloride through which is bubbled a controllable stream of fluid chlorine. When the milling action has continued as long as necessary to obtain the desired depth of metal removal (about 0.005"/hour with a saturated solution at 90° C.), the piece is removed from the system. The piece then needs only to be washed in water to completely remove the sodium silicate. The portion of the metal beneath the sodium silicate is not attacked and the design which had been painted on with the sodium silicate stands out in bold relief from the milled metal surface.

Generally the characteristic of the solvent which makes it effective within the practice of the present invention is that it contains an element with an extra available pair of electrons which coordinate with the available empty electron bands (usually "d") of the metal being milled.

The rate of the reaction of the chlorine in the phosphorus oxychloride is increased by using the chlorine under pressure to increase the concentration of the chlorine in solution. Raising the temperature will also result in a faster reaction rate although the rate of attack is found to increase more slowly with rising temperatures. It is noted, however, that the solubility of a gas in a liquid will decrease with temperature thereby decreasing concentration and slowing the reaction rate. The relative degree of these effects, i.e., heat on reaction rate per se and on concentration, should be balanced so as to achieve an optimum rate of milling. It is found that the maximum rate of removal can occur at a temperature of about 85-100° C. which is less than the boiling point of the phosphorus oxychloride. I further found that the application of pressure eliminates somewhat the bad effect of decreasing solubility with an increased temperature although extremely good results are obtained under a pressure of one atmosphere.

It is of course understood that the several embodiments

herein described are included to exemplify and not limit the invention and that any equivalent formulations are intended within the spirit of this invention especially as defined by the appended claims.

5. What is claimed is:

1. The chemical process for milling preselected portions of structural members consisting of ferrous metals and alloys comprising: immersing the preselected portion of the structural member into a nonaqueous solvent consisting essentially of phosphorus oxychloride; bubbling through the solvent a fluid oxidant selected from a group consisting of chlorine, bromine and iodine, until the surface has been milled its desired depth; and withdrawing said structural member from said solvent.

10 2. The chemical process for milling preselected portions of structural members consisting of ferrous metals and alloys comprising: immersing the preselected portion of the structural member into a heated nonaqueous solvent consisting essentially of phosphorus oxychloride; bubbling through the solvent a fluid oxidant selected from a group consisting of chlorine, bromine and iodine, until the surface has been milled its desired depth; and withdrawing said structural member from said solvent.

15 3. The chemical process for milling preselected portions of structural members consisting of ferrous metals and alloys comprising: immersing the preselected portion of the structural member into a nonaqueous solvent consisting essentially of phosphorus oxychloride; bubbling through the solvent a fluid oxidant consisting essentially of chlorine until the surface has been milled its desired depth; and withdrawing said structural member from said solvent.

20 4. The chemical process for milling preselected portions of structural members consisting of ferrous metals and alloys comprising: immersing the preselected portion of the structural member into a heated nonaqueous solvent consisting essentially of phosphorus oxychloride; bubbling through the solvent a fluid oxidant consisting essentially of chlorine, until the surface has been milled its desired depth; and withdrawing said structural member from said solvent.

25 5. The chemical process for milling preselected portions of structural members consisting of ferrous metals and alloys comprising: immersing the preselected portion of the structural member into a heated nonaqueous solvent consisting essentially of phosphorus oxychloride; bubbling a constant stream of chlorine until the surface has been milled its desired depth; and withdrawing said structural member from said solvent.

30 6. The chemical process for milling preselected portions of structural members consisting of ferrous metals and alloys comprising: immersing the preselected portion of the structural member into phosphorus oxychloride heated to a temperature less than its boiling point; bubbling a constant stream of chlorine until the surface has been milled its desired depth; and withdrawing said structural member from said solvent.

35 7. A process for chemically milling metallic members comprising preparing a bath consisting essentially of phosphorus oxychloride; heating said bath to a temperature of from 85-100° C.; immersing a metallic member into said heated bath; introducing a stream of an oxidizing fluid selected from the group consisting of bromine, iodine and chlorine, into said bath for diffused engagement with said member until said member has been milled a preselected depth; and withdrawing the milled metallic member from said bath.

40 8. A process for producing a milled metallic member according to a predetermined design having raised portions and sunken portions, the process comprising: painting with sodium silicate the surface portions of an unmilled metallic member corresponding to the raised portions of the predetermined design; drying said sodium silicate; immersing the sodium silicate painted metallic member into a heated bath consisting essentially of phos-

phorus oxychloride; flowing and maintaining a stream of a fluid oxidant through said bath for engagement with the unpainted surface portions of said member until said portions become the sunken portions of the predetermined design having a preselected depth; and withdraw- 5 ing said member from within said bath.

## References Cited in the file of this patent

## UNITED STATES PATENTS

2,756,373 Houtz ----- July 24, 1956  
FOREIGN PATENTS  
356,371 Germany ----- Dec. 7, 1921